

## UNITED STATES PATENT OFFICE

2,289,571

SINTERED ARTICLE AND METHOD OF  
MAKING THE SAMEAlfred L. Begehold, Detroit, Mich., assignor to  
General Motors Corporation, Detroit, Mich., a  
corporation of DelawareNo Drawing. Application September 6, 1940,  
Serial No. 355,609

4 Claims. (Cl. 75—22)

This invention relates generally to powder metallurgy and more particularly to powders made of brittle copper-tin alloys and the usage of the formed powders in the formation of sintered bronze articles.

It is well known to form articles such as bronze shings and other shapes from powdered copper and powdered tin which are mixed together with some graphite (with suitable binders if desired), briquetted and then sintered. The powdered copper available on the market for this purpose is expensive and costs considerably more in the market price of ingot copper. The same applies to the powdered tin.

One important object of this invention is to reduce the cost of sintered bronze articles.

Another object of this invention is to introduce of the tin and a portion of the copper required in the production of sintered bronze articles in the form of a brittle copper-tin alloy that is readily and economically comminuted or ground to the size of powder required.

It is also an object of this invention to provide economical method of making briquetted and sintered bronze articles that are stronger than articles made by briquetting and sintering under similar conditions a mixture of copper powder and tin powder.

Still another object of the present invention is to provide an economical method of producing an alloy powder of copper and tin that is especially adapted for use in the fabrication of sintered articles.

Other objects and advantages of my invention become more apparent as the description proceeds.

In accordance with a preferred embodiment of my invention, I provide a molten copper-tin alloy of such composition that the solidified alloy is quite brittle and friable, and hence may be readily comminuted or ground to any desired size. An alloy composed of about forty per cent tin and the balance substantially all copper has the necessary friability and at the present time is preferred. However, greater amounts of tin may be used to produce alloys having the desired ability to permit easy powdering. In general it is contemplated that about thirty-five to sixty per cent of tin and the balance substantially all copper may be employed.

The copper-tin alloy may be cast into suitable shapes and thereafter broken up in a suitable grinding or ball mill to the size of powder desired. The particular size in any case will depend on the use, but ordinarily it will be of a size such that it will all pass through a 100 mesh screen. In general, powder sizes on the same order as those now employed in making articles in briquetted and sintered powdered materials are usable. The copper-tin alloy powder is much

less costly than equivalent amounts of copper and tin as separate or non-alloyed powders. This is due largely to the ease with which the alloy material is broken up into powder as compared with the cost of powdering copper and tin separately.

In the formation of sintered and briquetted bronze articles in accordance with a preferred embodiment of the invention all of the tin required in the final article is introduced in the form of the brittle copper-tin alloy powder. The required amount of the copper-tin alloy powder is then intimately mixed with copper powder and a small amount of graphite. The powder mixture is then compressed or briquetted into the form desired and thereafter sintered. Briquetting pressures and sintering temperatures and times on the same order as those employed in making briquetted and sintered articles from copper and tin powders may be used. Preferably the sintering operation is carried out under non-oxidizing conditions, as in an atmosphere containing carbon monoxide or other reducing gas or gases.

The copper-tin alloy powder in addition to reducing the cost of the sintered article by a less costly source of the tin that is necessary and by a less costly source of a portion of the copper required, also assists in making a stronger sintered material than where separate copper and tin powders are used. This is due to the fact that where the tin is supplied in the form of the copper-tin alloy powder no voids, such as would be formed by melting of the tin particles and migration of the tin into the copper, are produced during sintering. In the present invention as the sintering operation proceeds, some of the tin migrates from the copper-tin alloy particles into the copper particles, leaving behind the copper-tin alloy particles of reduced tin content. This results in a sintered article having less discontinuity of structure than where separate copper and tin powders are employed. The migration of the tin from the regions of high tin content into those of no tin content increases the strength of the particles or regions low in tin and eliminates the brittleness from the particles which were originally high in tin. The diffusion can be carried out to the point where the composition and structure are uniform throughout. A ductile material or article is thus produced that is stronger and more homogeneous than an article of similar analysis made by briquetting and sintering under similar conditions a mixture of separate copper and tin powders.

In some applications the copper-tin alloy powder may be intimately mixed with other metal or alloy powders in addition to the copper powder and used in the formation of sintered articles.

In addition to the above described advantages resulting from forming bronze articles by a mixture of copper and copper-tin alloy powders, it appears that the frictional or stripping pressures are substantially lower than with briquettes formed of a mixture of copper and tin powders. Lower stripping pressures mean less wear of the dies used in the briquetting operation and permit articles of greater lengths to be briquetted.

For illustrative purposes the following specific examples of procedure in accordance with the invention may be given.

Twenty-five parts of an alloy powder composed of forty per cent tin and the balance copper was intimately mixed with seventy-five parts of copper powder, briquetted under a pressure of 50,000 pounds per square inch, and thereafter sintered at a temperature of 1500° F. in a non-oxidizing atmosphere containing carbon monoxide. The powders were of a size such that all would pass through a 150 mesh screen and about eighty-five per cent through a 200 mesh screen. A strong sintered bronze article was produced.

In another case ten parts of a nickel-silicon alloy composed of twenty-eight per cent silicon, about two per cent iron and the balance copper, were thoroughly mixed with five parts of the forty per cent copper-tin alloy powder and eighty-five parts of copper powder. The mixture was briquetted under a pressure of 50,000 pounds per square inch and sintered under non-oxidizing conditions at a temperature of 1700° F. The powders were of a size such that all would pass through a 150 mesh screen and about eighty-five per cent through a 200 mesh screen. The sintered article had a strength of about 40,000 pounds per square inch and had good properties as regards score resistance.

In some cases it may be desirable that the copper-tin alloy powder be of a different size than the copper powder. In making articles by briquetting and sintering it is often desirable to provide a certain amount or proportion of the powder of a very fine size. Due to the ease with which the copper-tin alloy material can be broken up into a very fine powder, the alloy powder may conveniently supply the amount of extremely fine powder required.

Various changes and modifications of the preferred embodiments of my invention described herein may be made without departing from the principles of my invention and I do not intend to limit the patent granted thereon except as necessitated by the prior art.

I claim:

1. The method of making a briquetted and sintered bronze article which comprises; forming a copper-tin alloy powder consisting of 35% to 60% tin and the balance substantially all copper; mixing a relatively small amount of said copper-tin alloy powder sufficient to provide the required tin content in the finished article, with copper powder; briquetting the mixture of the copper-tin alloy powder and the copper powder; and sintering said briquetted powder mixture at a sintering temperature below the melting point of the copper powder and at least as high as the minimum temperature necessary to fuse entirely the copper-tin alloy powder and for a time sufficient to cause migration of tin from the copper-tin alloy powder particles into the copper powder particles until the tin content in the copper-tin

alloy powder particles is lowered to the point where they become ductile to thereby form a ductile, sintered bronze article consisting of copper and tin and having less discontinuity of structure and greater strength than sintered bronze articles of similar analysis formed by briquetting and sintering a mixture of copper powder and tin powder.

2. The method of making a briquetted and sintered bronze article which comprises, forming a brittle copper-tin alloy material containing 35% to 60% tin and the balance substantially all copper, forming a powder of said copper-tin alloy of a size such that it will at least pass through a 100 mesh screen, mixing a relatively small amount of said copper-tin alloy powder sufficient to provide the amount of tin desired in the bronze with the necessary amount of copper powder, compressing said mixture of powder under high pressure into the shape desired, a sintering said briquette at a temperature of about 1500° F. in a non-oxidizing atmosphere and for a time sufficient to cause migration of the tin from the copper-tin alloy particles to the copper particles and to form a strong ductile sintered bronze article of homogeneous structure throughout.

3. The method of making a briquetted and sintered article which comprises forming a brittle copper-tin alloy powder containing 35% to 60% tin and the balance substantially all copper, mixing a relatively small proportion of said copper-tin alloy powder with a relatively large proportion of other metallic powder to provide the tin desired in the final article, briquetting said powder mixture, and sintering said briquette at a sintering temperature at least as high as the minimum temperature necessary to provide a molten component in the copper-tin alloy powder and for a time sufficient to cause migration of the tin into the other metallic powder particles until the tin becomes substantially uniform and diffused throughout the article whereby a strong ductile sintered article of homogeneous structure is produced.

4. The method of making a briquetted and sintered bronze article which comprises, forming a brittle copper-tin alloy containing about 40% tin and the balance substantially all copper, powdering said brittle copper-tin alloy to a size such that it will pass through a 150 mesh screen, mixing about twenty-five parts of said brittle copper-tin powder with about seventy-five parts of copper powder of a size such that it will pass through a 150 mesh screen, all of the tin in the final article being supplied by the brittle copper-tin alloy powder, briquetting said powder mixture under a pressure of around 50,000 pounds per square inch, and sintering said briquette at a temperature of about 1500° F. in a non-oxidizing atmosphere until tin from the copper-tin alloy powder particles has diffused substantially uniformly through the copper particles and a strong, ductile bronze article consisting of about 90% copper and 10% tin is produced having greater strength and less discontinuity of structure than sintered bronze articles of similar analysis formed by briquetting and sintering under similar pressure and temperature conditions a mixture of copper powder and tin powder.

ALFRED L. BOEGEHOOLD.